# EUROPEAN PATENT SPECIFICATION

(11) **EP 0 618 023 B1**
(45) Date of publication and mention of the grant of the patent: **17.06.1998**
(21) Application number: 92920028.5
(22) Date of filing: 22.09.1992
(51) Int. Cl.: B22D 11/04, B22D 11/16

(54) **CASTING CONTINUOUS SLAB IN OSCILLATED MOLD WITH HORIZONTALLY RETRACTABLE WALLS**
STRANGGIESSEN VON BRAMMEN IN OSZILLIERENDER KOKILLE MIT HORIZONTAL ZURüCKZIEBAREN WÄNDEN
COULEE CONTINUE DE BRAMES EN LINGOTIERE OSCILLEE AVEC RETRAIT HORIZONTAL DES PAROIS

(43) Date of publication of application: 05.10.1994
(73) Proprietor: KAWASAKI STEEL CORPORATION, Kobe-shi Hyogo-ken 651 (JP)
(72) Inventor: ITOYAMA, Seiji;, Technical Research Division of, Chuo-ku, Chiba-shi;, Chiba-ken 260 (JP); TOZAWA, Hirokazu;, Technical Research Division of, Chuo-ku, Chiba-shi;, Chiba-ken 260 (JP); TAKEUCHI, Shuji;, Technical Research Division of, Chuo-ku, Chiba-shi;, Chiba-ken 260 (JP); SORIMACHI, Kenichi;, Technical Research Division, Chuo-ku, Chiba-shi;, Chiba-ken 260 (JP)
(74) Representative: Grünecker, Kinkeldey, Stockmair & Schwanhäusser Anwaltssozietät
(86) International application number: JP9201205
(87) International publication number: WO9406583

(56) References cited:
- EP-A- 0 372 506
- EP-A- 0 570 935
- WO-A-85/04125
- JP-A- 2 290 656
- JP-A- 3 099 756
- JP-A- 3 297 546
- JP-A- 4 143 057
- JP-A-64 018 553
- US-A- 3 700 024

## Description

### Technical Field

The present invention relates to a casting process for continuous castings, capable of obtaining the castings reduced in the depths of oscillation marks and suppressed in segregation at oscillation mark trough portions, in a continuous casting method, particularly, a vertical continuous casting method for metal.

### Background Art

Conventionally, for the purpose of eliminating the repairing work for the surfaces of continuous castings, there has been proposed a technique of oscillating a vertical mold for reducing or preventing positive segregations at oscillation mark trough portions on the surfaces of the castings, particularly, in casting stainless steel (SUS 304). For example, Japanese Patent Laid-open No. hei 2-290656 has disclosed such a technique that, in a continuous casting mold of a type forming a casting space with two pairs of mold wall surfaces, a pair of the mold wall surfaces are relatively separated from each other only for a negative strip time zone in vertical oscillation or for a mold descending time zone.

This technique is recognized to be considerably effective as compared with a case of giving only simple vertical oscillation. However, as a result of an experiment, it is seen that the technique is not much effective for such a case that the oscillation frequency 〈f〉 of the mold is small. Further, in the above technique, the consumption of mold powder is reduced, thereby causing the breakout due to sticking. Accordingly, on the contrary, there is arisen an inconvenience of obstructing the stable casting.

Conventionally, the mechanism and cause of generating the segregations at oscillation mark trough portions were considered as follows: namely, the negative pressure is generated within a liquid phase lubricating film between the mold and the solidified shell due to oscillation of the mold;and due to this negative pressure, the non-solidified and concentrated molten steel between dendrites of the solidified surface layer permeates onto the surface of the shell.

However, as a result of the examination on the segregated portions of the casting by the present inventors, it was revealed that the segregation is generated in accordance with such a mechanism that the continuous growth of the solidified shell is obstructed by breaking of the shell due to a tensile force applied thereto and by buckling due to a compressive force, and thereby the concentrated liquid flows out from the broken portions or buckled portions of the shell to the surface of the shell. Accordingly, for preventing the segregation, it is effective to prevent the breaking or the buckling of the shell at the beginning of the solidification, that is, to simultaneously reduce the tensile force and the compressive force applied to the shell.

An object of the present invention is to provide a process of withdrawing the continuous castings wherein, even in the low cycle condition that the oscillation frequency 〈f〉 of the mold is small, the segregations at oscillation mark trough portions on the surfaces of the castings are significantly reduced to the degree equivalent to that in the high cycle condition, and also the stable casting is made possible.

### Disclosure of the Invention

In a first mode of the present invention, defined in claim 1, there is provided a casting process for continuous castings characterized by vertically oscillating a vertical continuous casting mold forming a casting space with two pairs of mold wall surfaces; and simultaneously repeating a series of actions composed of separating at least a pair of mold wall surfaces from a solidified shell at any period in each specified time zone within a positive strip time zone and a negative strip time zone, and of making the separated mold wall surfaces close to the solidified shell within the other time zones.

In a second mode of the invention according to independent claim 3, there is provided a casting process for continuous castings characterized by performing the casting under the condition of only a positive strip tame zone, while vertically oscillating a vertical continuous casting mold forming a casting space with two pairs of mold wall surfaces; and repeating a series of actions composed of separating at least a pair of mold wall surfaces from a solidified shell at any period in each specified time zone within a mold ascending period and a mold descending period, and making the separated mold wall surfaces close to the solidified shell within the other time zones in the mold ascending period and the descending period

### Brief Description of the Drawings

Fig. 1 is a graph showing the changes in the vertical oscillating velocity of a mold and the horizontal displacement of the mold walls with time according to an embodiment of the present invention;
Fig. 2 is a graph showing the changes in the vertical oscillating velocity of a mold and the horizontal displacement of the mold walls with time according to another embodiment of the present invention;
Fig. 3 is a schematic perspective view showing a mold horizontally moving apparatus used in the embodiments of the present invention;
Fig. 4 is a typical view showing an oscillation mark and a segregated layer;
Fig. 5 is graphs showing an oscillation waveform of the conventional mold, and the retarding and advancing timings thereof; and
Fig. 6 is a typical view showing the portion between the mold wall and the solidified shell.

### Best Mode for Carrying Out the Invention

As shown in Fig. 1, when a mold reaches the uppermost point, the vertical velocity Vm of the mold becomes 0. Subsequently, as the mold is started to be descended, the velocity Vm is gradually increased. Thus, when the mold reaches the lowermost point, the velocity Vm becomes 0. When the mold is started to be ascended again, the velocity Vm of the mold is increased. Also, in terms of the relative relationship between the vertical velocity of the mold and the withdrawing velocity Vc of the casting, the time for which the vertical velocity Vm of the mold is smaller than the withdrawing velocity Vc is referred to as " negative strip time T_{N} .

In vertical oscillation of the mold as shown in Fig. 1, at any period in a time zone from the time tl to t2 for which the $\text{relative velocity (=Vm-Vc)}$ is larger within a positive strip time Tp for which the solidified shell is applied with a tensile force, at least a pair of mold walls are horizontally retracted in a manner to be relatively separated from the solidified shell, to be thus opened at the position of Xo. In absence of the negative strip time T_{N} (T_{N} = 0), as shown in Fig. 2, at a ny period in a time zone from the time t₄ to t₅ for which the relative velocity is larger within a mold ascending time, at least a pair of mold walls are retracted in a manner to be relatively separated from the solidified shell, to be thus opened at the position of Xo.

Thus, as shown in Fig. 6, a distance between a mold wall 9 and a solidified shell 12 is increased from Xs to Xo, so that a mold powder 10 on a molten steel 11 is made to sufficiently flow in a gap between the mold wall 9 and the solidified shell 12 to thereby reduce the frictional force between the mold wall 9 and the solidified shell 12. In addition, the arrow of Y indicates the direction of withdrawing the casting.

In Fig. 1, at any period in a subsequent time zone from the time t3 to t4 for which the relative velocity is smaller within the negative strip time T _{N} for which the compressive force is applied to the shell, the mold walls are relatively separated from the solidified shell, to be thus opened at the position of Xo. In absence of no negative strip time T_{N} (T_{N} = 0), as shown in Fi g. 2, at any period in a time zone from the time t2 to t3 for which the relative velocity is smaller in a mold descending time, at least a pair of mold walls are retarded in a manner to be relatively separated from the solidified shell, to be thus opened at the position of Xo. In absence of the negative strip, since the relative velocity between the mold and the solidified shell is usually directed upwardly, it is considered that the shell is not applied with the compressive force. However, since the solidified shell at the meniscus portion within the mold is continuously grown and the position thereof is made constant, the shell is applied with the compressive force even in the case of T _{N} = 0.

For the time zones other than those described above, that is, for the time zones from the time t2 to t3 and from the time t4 to t5 in Fig. 1, and the time zones from the time t1 to t2 and from the time t3 to t4 in Fig. 2, the mold walls are advanced to be close to the solidified shell, to be thus closed at the position of Xs. Namely, the distance X between the mold and the solidified shell is changed from Xo to Xs. In the case of giving the horizontal oscillation to the mold for changing the distance between the mold wall surfaces and the solidified shell, particularly, the frictional force applied to the initial solidified shell of the meniscus portion can be calculated, under the consideration of the frictional force between the mold and the solidified shell, as the shear force applied between the mold and the solidified shell by the following equation:$\text{F = A · µ (dV / dX)}$ wherein
- A :: contact area between mold and solidified shell
- µ :: viscosity of mold powder flown in space between mold wall and solidified shell
- dV:: relative velocity between mold wall and solidified shell (=Vm-Vc)
- X :: distance between mold and solidified shell
As is apparent from the above equation (1), the frictional force F applied to the solidified shell is reduced at the period for which the distance X between the mold and the solidified shell is enlarged. Namely, according to the present invention, it is possible to significantly reduce the tensile force and the compressive force applied to the shell of the meniscus portion at the beginning of the solidification. Consequently, the continuity of the solidified shell is held, thereby making it possible to narrow the depths of the oscillation marks, and to reduce the possibility of generating the segregation at the oscillation mark trough portions as compared with the conventional technique.

The effect describe above is not much dependent on the vertical oscillation waveform and a waveform for horizontally advancing/retracting (closing/opening) the mold walls (hereinafter, referred to as "horizontal oscillation"), and which is similarly effective in the cases of the non-sinusoidal wave or triangular wave other than the vertical oscillation of the sinusoidal wave and the horizontal wave of the trapezoidal wave as shown in Fig. 1. In addition, for preventing molten steel from permeating in the gaps at the mold corners thereby bringing about a fear of causing the sticking induced breakout, the amplitude of the horizontal oscillation is preferably within the range of 1mm or less.

Hereinafter, the present invention will be described in detail with reference to examples.

### Example 1

As shown in Fig. 3, a horizontal oscillator generally used for a slab continuous casting machine has a mechanism of clamping mold short sides 2 with mold long sides 1 through short side clamping springs 3. In the present invention, there is provided a hydraulic circuit for opening/closing a short side clamping hydraulic cylinder 4, so that the long sides 1 of the mold is moved by opening and closing the short side clamping hydraulic cylinder 4 through upper and lower solenoid valves 5 and 6 provided in a hydraulic circuit. Numeral 7 indicates a hydraulic motor and numeral 8 is a hydraulic tank. If the gaps between the long sides and short sides of the mold are made excessively larger, molten steel permeates in the gaps, thereby causing the trouble. Accordingly, the retracted amount of the long sides of the mold is within the range of 1mm or less.

The casting of stainless steel (SUS 304) was continuously cast using the above horizontal oscillator for horizontally oscillating the mold walls as shown in Fig. 3. In the above casting, from the depth d₁, at an oscillation mark 13 (see Fig. 4) and the segregation layer depth d2 at the segregation mark portion on the surface of the casting, the segregation layer thickness (d2 -dl) at the oscillation mark portion was obtained. Thus, the examination was made for the above segregation layer thickness (d2 -dl) and the segregation layer depth d2. For comparison, the examinations were made for the cases of generating only the vertical oscillation (sinusoidal wave) according to the conventional manner; and of generating such oscillating waves as shown in Figs. 5(a) and 5(b) disclosed in Japanese Patent Laid-open No. Hei 2-290656. In the above, Fig. 5(a) shows the case of moving the mold walls backward during the period when the oscillation of the mold lies in the negative strip time. Besides, Fig. 5(b) shows the case of retarding the mold in the mold descending period. In addition, the casting condition of the present invention is as follows: withdrawing velocity Vc of castings= 1.2/min; mold vertical oscillating frequency f = 150 times/min; amplitude S = 5.3mm; vertical oscillating waveform = sinusoidal curve; horizontal oscillating amplitude =0.3mm; horizontal oscillating pattern is trapezoidal wave (see Fig. 1). Further, the mold wall opening/closing timing is closed (at the position of Xs) for a period from 105 ° to 130 ° (from the time t2 to t3 in Fig. 1) in terms of angle conversion (zero angle, when V m is positively maximized), and a period from 240° to 275 ° (from the time t4 to t5 in Fig. 1), and is opened (at the position of Xo) for the other periods. The moving velocity from the opening to the closing, or the closing to the opening was specified at 50mm/sec. In addition, as the mold power, there was used a lubricant having a viscosity of 1.1 poise at 1300 ° C and the solidification temperature of 900° C.

### Example 2

Next, for the case of no negative strip time (T _{N} 0), the test was carried out in the same manner as in Example 1, except that the amplitude S of the mold vertical oscillation was 2.0mm, and the horizontal opening and closing timing was closed in the period from 110 ° to 160 ° (from the time t1 to t2 in Fig. 2) and in a period from 250° to 290 ° (from the time t3 to t4 in Fig. 2), and was opened in the other periods.

The results obtained in Examples 1 and 2 are shown in Table 1 as compared with the conventional manner. It becomes apparent from Table 1 that, as compared with the conventional manner, the present invention makes it possible to significantly reduce the rate of generating the segregations at the oscillation trough portions to the degree of being almost zero.

### Industrial Applicability

By provision of a mold oscillation method of horizontally opening and closing (retracting and advancing) the mold walls from and to the solidified shell according to the mold vertical oscillating timing for extremely reducing the compressive force and the tensile force applied to the initial solidified shell, it is possible to significantly reduce the segregations at the oscillation trough portions on the surface of the casting. As a result, the following effects can be obtained:
(1) By eliminating the need of performing the casting under the high cycle mold oscillating condition having a fear of causing the generation of the sticking induced breakout, it is possible to reduce the trouble in productivity.
(2) In the case of stainless steel (SUS 304), since it is possible to reduce the amount to be cut by a grinder for removing the segregations before the heating and rolling processes as in the conventional manner, and further to supply the casting to the next process with no repairing in the specific case, the improvement in yield can be expected.

## Claims

1. A method for continuous vertical casting of molten metal through a mold so as to form a casting having an outer surface in the form of a solidified metallic shell, said mold having a casting space formed by a first pair of opposed walls and a second pair of opposed walls, said first and second walls being perpendicular to each other and in contact with said shell, one of said first and second pairs of opposed walls movable towards and away from each other and from contact with said shell, the method comprising the steps of:
vertically and cylindrically oscillating said mold so as to define a mold ascending travel period and a mold descending travel period, said ascending travel period corresponding to a period of time said mold requires to upwardly travel from a lowermost oscillation point to an uppermost oscillation point, and said descending travel period corresponding to a successive period of time said mold requires to downwardly travel from said uppermost oscillation point back to said lowermost oscillation point, said mold having a maximum upward velocity during said ascending travel period corresponding to a midpoint between said uppermost and uppermost oscillation points, and said mold having a maximum downward velocity during said descending travel period corresponding to a midpoint between said uppermost and lowermost oscillation points, said uppermost and lowermost points corresponding to a mold position where said mold velocity is zero due to said mold changing between an upwardly and downwardly travel direction, said casting having a downward direction and a constant withdrawal velocity, said ascending travel period having a portion thereof wherein said mold has a vertical velocity that is greater than said withdrawal velocity of said casting and said descending travel period having a portion thereof wherein said mold has a vertical velocity that is greater than said withdrawal velocity of said casting;
retracting said movable walls from each other and from said casting shell when said mold vertical velocity is operable during said portion of said ascending travel period where said vertical velocity of said mold is greater than said withdrawal velocity of said casting; and
retracting said movable walls from each other and from said casting shell when said mold vertical velocity is operable during said portion of said descending period where said vertical velocity of said mold is greater than said withdrawal velocity of said casting.

2. The method of continuously vertical casting molten metal of claim 1, further including the step of injecting a mold powder between said movable mold walls and said shell of said casting when said mold walls are retracted, thereby reducing the frictional force between said movable mold walls and said shell.

3. A method for continuous vertical casting of molten metal through a mold so as to form a casting having an outer surface in the form of a solidified metallic shell, said mold maximum downward velocity during said descending travel period corresponding to a midpoint between said uppermost and lowermost oscillation points, said uppermost and lowermost points corresponding to a mold position where said mold velocity is zero due to said mold changing between an upwardly and downwardly travel direction,
wherein said mold vertical velocity during successive ascending and descending travel periods defines a positive time strip and a negative time strip, said positive and negative time strips each defining a relationship between the vertical velocity of said mold and a withdrawal velocity of said casting, each of said positive and negative time strips having a starting time and a finishing time, said starting time of said positive time strip corresponding to a finishing time of said negative time strip and said finishing time of said positive time strip corresponding to a starting time of said negative time strip, each of said starting and finishing times of said positive and negative time strips corresponding to a point where said mold has a speed equivalent to a speed of said casting and where a relative velocity between said mold and said casting is zero, said positive time strip defined as a period of time within said ascending and descending travel periods wherein said mold vertical velocity is relatively greater than said withdrawal velocity of said casting and said negative time strip defined as a period of time within said ascending and descending travel periods wherein said mold vertical velocity is relatively less than said withdrawal velocity of said cast metal;
retracting said movable walls away from each other and from contact with said shell when said mold vertical velocity is operably within said positive time strip, said walls being opened at a first period of time corresponding to where said mold vertical velocity is between that of said starting point of said positive time strip and that of said mold maximum vertical velocity within said positive time strip,
said movable walls being closed towards each other and into contact with said shell at a second period of time corresponding to where said mold vertical velocity is between that of said maximum vertical velocity within said positive time strip and that of said finishing point of said positive time strip, said opening and closing of said walls at said first and second periods of time occurring at equal velocities within said positive time strip; then
retracting said movable walls away from each other and from contact with said shell when said mold vertical velocity is operably within said negative time strip, said walls being opened at a third period of time corresponding to where said mold vertical velocity is between that of said starting point of said negative time strip and that of said mold maximum vertical velocity within said negative time strip,
said movable walls being closed towards each other and into contact with said shell at a fourth period of time corresponding to where said mold vertical velocity is between that of said maximum vertical velocity within said negative time strip and that of said finishing point of said negative time strip, said opening and closing of said walls at said third and fourth periods of time occurring at equal velocities within said negative time strip.

## Patentansprüche

1. Verfahren zum Vertikal-Stranggießen von Metallschmelze durch eine Form, um ein Gußteil mit einer Außenfläche in Gestalt eines erstarrten Metallmantels zu bilden, wobei die Form einen Gußteilraum besitzt, der durch ein erstes Paar einander gegenüberliegender Wände und ein zweites Paar einander gegenüberliegender Wände gebildet wird, welche ersten und zweiten Wände senkrecht zueinander mit dem Mantel in Berührung stehen, eines der ersten und zweiten Paare einander gegenüberliegender Wände zueinander hin und voneinander weg und aus der Berührung mit dem Mantel bewegbar ist, und das Verfahren die Schritte umfaßt:
vertikales und zylindrisches Oszillieren der Form, um so einen Formaufsteige-Laufzeitraum und einen Formabsteige-Laufzeitraum zu bestimmen, welcher Aufsteige-Laufzeitraum einem Zeitraum entspricht, welchen die Form braucht, um von einem untersten Oszillationspunkt zu einem obersten Oszillationspunkt aufwärts zu laufen, und der Absteige-Laufzeitraum einem darauffolgenden Laufzeitraum entspricht, den die Form braucht, um von dem obersten Oszillationspunkt zurück zu dem unteren Oszillationspunkt zu laufen, wobei die Form während des Aufsteige-Laufzeitraumes eine maximale Aufsteige-Geschwindigkeit besitzt, die einer Mittelstelle zwischen dem obersten und dem untersten Oszillationspunkt entspricht, und die Form während des Absteige-Laufzeitraumes eine maximale Absteige-Geschwindigkeit besitzt, die einer Mittelstelle zwischen dem obersten und dem untersten Oszillationspunkt entspricht, und der oberste und der unterste Punkt jeweils einer Position der Form entsprechen, bei der die Formgeschwindigkeit Null ist, da die Form zwischen einer Aufwärts- und einer Abwärts-Laufrichtung wechselt, während das Gußteil eine abwärts gerichtete und konstante Abzieh-Geschwindigkeit besitzt, der Absteige-Laufzeitraum einen Abschnitt enthält, bei dem die Form eine Vertikal-Geschwindigkeit besitzt, die höher als die Abzieh-Geschwindigkeit des Gußteils ist, und der Absteige-Laufzeitraum einen Abschnitt enthält, bei dem die Form eine Vertikal-Geschwindigkeit besitzt, die höher als die Abzieh-Geschwindigkeit des Gußteils ist;
Zurückziehen der bewegbaren Wände voneinander und Abziehen derselben von dem Gußteilmantel, wenn die Vertikal-Geschwindigkeit der Form wahrend des Abschnitts des Aufsteige-Laufzeitraums betätigbar ist, bei dem die Vertikal-Geschwindigkeit der Form größer als die Abzieh-Geschwindigkeit des Gußteils ist; und
Zurückziehen der bewegbaren Wände voneinander und von dem Gußteilmantel, wenn die Vertikal-Geschwindigkeit der Form während des Abschnittes des Absteige-Laufzeitraums betätigbar ist, bei dem die Vertikal-Geschwindigkeit der Form höher als die Abzieh-Geschwindigkeit des Gußteils ist.

2. Verfahren zum Vertikal-Stranggießen von Metallschmelze nach Anspruch 1, das weiter den Schritt des Einführens eines Formpulvers zwischen die bewegbaren Formwände und den Mantel des Gußteils enthalt, wenn die Formwände zurückgezogen werden, um dadurch die Reibkraft zwischen den bewegbaren Formwänden und dem Mantel herabzusetzen.

3. Verfahren zum Vertikal-Stranggießen von Metallschmelze durch eine Form, um so ein Gußteil mit einer Außenfläche in Gestalt eines erstarrten Metallmantels zu bilden, wobei die maximale Formgeschwindigkeit nach unten wahrend des Absteige-Laufzeitraumes einem Mittelpunkt zwischen dem obersten und dem untersten Oszillationspunkt entspricht, der oberste und der unterste Punkt jeweils einer Formposition entspricht, wo die Formgeschwindigkeit Null ist, da die Form zwischen einer Aufwärts- und einer Abwärts-Laufrichtung wechselt,
die Vertikal-Geschwindigkeit der Form wahrend aufeinanderfolgender Aufsteige- und Absteige-Laufzeiträume eine positive Abstreifzeit bzw. eine negative Abstreifzeit bestimmt, die positiven und negativen Abstreifzeit jeweils eine Beziehung zwischen der Vertikal-Geschwindigkeit der Form und einer Abzieh-Geschwindigkeit des Gußteils bestimmen, jede der positiven und negativen Abstreifzeiten einen Beginn-Zeitpunkt und einen Beendigungs-Zeitpunkt besitzt, der Beginn-Zeitpunkt der positiven Abstreifzeit einem Beendigungs-Zeitpunkt der negativen Abstreifzeit und der Beendigungs-Zeitpunkt der positiven Abstreifzeit einem Beginn-Zeitpunkt der negativen Abstreifzeit entspricht, jeder der Beginn- und Beendigungs-Zeitpunkte der positiven und der negativen Abstreifzeiten einem Punkt entspricht, bei dem die Form eine einer Geschwindigkeit des Gußteils äquivalente Geschwindigkeit besitzt und eine Relativgeschwindigkeit Null zwischen der Form und dem Gußteil, die positive Abstreifzeit bestimmt ist als ein Zeitraum innerhalb der Aufsteige- bzw. Absteige-Laufzeiträume, bei dem die vertikale Geschwindigkeit der Form relativ größer als die Abzieh-Geschwindigkeit des Gußteils ist, und die negative Abstreifzeit bestimmt ist als ein Zeitraum innerhalb der Aufsteige- und der Absteige-Laufzeiträume, bei dem die vertikale Formgeschwindigkeit relativ geringer als die Abzieh-Geschwindigkeit des Gußteils ist;
mit Zurückziehen der bewegbaren Wände voneinander und aus der Berührung mit dem Mantel, wenn die Vertikal-Geschwindigkeit der Form innerhalb der positiven Abstreifzeit betätigbar ist, welche Wände in einem ersten Zeitraum geöffnet werden, der dem entspricht, in dem die Vertikal-Geschwindigkeit der Form zwischen der am Beginnpunkt der positiven Abstreifzeit und der der maximalen vertikalen Formgeschwindigkeit innerhalb der positiven Abstreifzeit liegt, die bewegbaren Wände aufeinander zu und in Berührung mit dem Mantel in einem zweiten Zeitraum geschlossen werden, der dem entspricht, in dem die Vertikal-Geschwindigkeit der Form zwischen der der maximalen Vertikal-Geschwindigkeit innerhalb der positiven Abstreifzeit und der des Beendigungs-Zeitpunktes der positiven Abstreifzeit liegt, das Öffnen und Schließen der Wände bei den ersten und zweiten Zeiträumen mit gleichen Geschwindigkeiten innerhalb der positiven Abstreifzeit auftritt; und dann
mit Zurückziehen der bewegbaren Wände voneinander weg und aus der Berührung mit dem Mantel, wenn die vertikale Formgeschwindigkeit innerhalb der negativen Abstreifzeit betätigbar ist, wobei die Wände in einem dritten Zeitraum geöffnet werden, der dem entspricht, in dem die vertikale Formgeschwindigkeit zwischen der des Beginnpunktes der negativen Abstreifzeit und der der maximalen vertikalen Formgeschwindigkeit innerhalb der negativen Abstreifzeit liegt,
wobei die bewegbaren Wände zueinander hin und in Berührung mit dem Mantel in einem vierten Zeitraum geschlossen werden, der dem entspricht, wo die vertikale Formgeschwindigkeit zwischen der der maximalen Vertikal-Geschwindigkeit innerhalb der negativen Abstreifzeit und der des Beendigungs-Zeitpunktes der negativen Abstreifzeit liegt, und das Öffnen und Schließen der Wände in den dritten und vierten Zeiträumen bei gleichen Geschwindigkeiten innerhalb der negativen Abstreifzeit auftritt.

## Revendications

1. Procédé de coulée verticale continue de métal en fusion dans une lingotière de façon à former une coulée présentant une surface extérieure ayant la forme d'un moule mince métallique solidifié, ladite lingotière présentant un espace de coulée formé grâce à une première paire de parois opposées et une seconde paire de parois opposées, lesdites premières et secondes parois étant perpendiculaires et en contact avec ledit moule mince, une paire desdites première et seconde paire de parois opposées pouvant se déplacer pour se rapprocher et s'éloigner l'une de l'autre et cesser d'être en contact avec ledit moule mince, le procédé comprenant les étapes suivantes :
oscillation verticale et cylindrique de ladite lingotière de façon à définir une période de déplacement ascendant de la lingotière et une période de déplacement descendant de la lingotière, ladite période de déplacement ascendant correspondant à une période de temps nécessaire à la lingotière pour se déplacer vers le haut à partir d'un point d'oscillation le plus bas jusqu'à un point d'oscillation le plus haut, et ladite période de déplacement descendant correspondant à une période de temps successive nécessaire à la lingotière pour se déplacer vers le bas à partir dudit point d'oscillation le plus haut et revenir audit point d'oscillation le plus bas, ladite lingotière ayant une vitesse maximum vers le haut au cours de ladite période de déplacement ascendant correspondant à un point médian entre lesdits points d'oscillation le plus haut et le plus bas, et ladite lingotière ayant une vitesse maximum vers le bas au cours de ladite période de déplacement descendant correspondant à un point médian entre lesdits points d'oscillation le plus haut et le plus bas, lesdits points le plus haut et le plus bas correspondant à une position de la lingotière pour laquelle ladite vitesse de la lingotière est nulle en raison du changement pour ladite lingotière d'un sens de déplacement vers le haut à un sens de déplacement vers le bas, ladite coulée présentant un sens dirigé vers le bas et une vitesse constante de retrait, ladite période de déplacement ascendant présentant une partie dans laquelle ladite lingotière a une vitesse verticale qui est supérieure à ladite vitesse de retrait de ladite coulée et ladite période de déplacement descendant présentant une partie dans laquelle ladite lingotière a une vitesse verticale qui est supérieure à ladite vitesse de retrait de ladite coulée ;
rétraction desdites parois mobiles l'une par rapport à l'autre et par rapport audit moule mince de coulée lorsque la vitesse verticale de la lingotière peut s'appliquer au cours de ladite partie de ladite période de déplacement ascendant lorsque ladite vitesse verticale de ladite lingotière est supérieure à ladite vitesse de retrait de ladite coulée ; et
rétraction desdites parois mobiles l'une par rapport à l'autre et par rapport audit moule mince de coulée lorsque la vitesse verticale de la lingotière peut s'appliquer au cours de ladite partie de ladite période de déplacement descendant lorsque ladite vitesse verticale de ladite lingotière est supérieure à ladite vitesse de retrait de ladite coulée.

2. Procédé de coulée verticale continue de métal en fusion selon la revendication 1, comportant en outre l'étape consistant à injecter une poudre de moulage entre lesdites parois de lingotière mobiles et ledit moule mince de ladite coulée lorsque lesdites parois de lingotière sont rétractées, ce qui réduit la force de frottement entre ledit moule mince et lesdites parois mobiles.

3. Procédé de coulée verticale continue de métal en fusion dans une lingotière de façon à former une coulée présentant une surface extérieure sous la forme d'un moule mince métallique solidifié, ladite vitesse descendante maximum de la lingotière au cours de ladite période de déplacement descendant correspondant à un point médian entre lesdits points d'oscillation le plus haut et le plus bas, lesdits points le plus haut et le plus bas correspondant à une position de la lingotière pour laquelle ladite vitesse de la lingotière est nulle en raison du changement pour la lingotière d'un sens de déplacement vers le haut à un sens de déplacement vers le bas,
dans lequel ladite vitesse verticale de la lingotière au cours des périodes successives de déplacement ascendant et descendant définit une bande de temps positive et une bande de temps négative, lesdites bandes de temps positive et négative définissant chacune une relation entre la vitesse verticale de ladite lingotière et une vitesse de retrait de ladite coulée, chacune desdites bandes de temps positive et négative ayant un moment de début et un moment de fin, ledit moment de début de ladite bande de temps positive correspondant à un moment de fin de ladite bande de temps négative et ledit moment de fin de ladite bande de temps positive correspondant à un moment de début de ladite bande de temps négative, chacun desdits moments de début et de fin desdites bandes de temps positive et négative correspondant à un point pour lequel ladite lingotière a une vitesse équivalente à une vitesse de ladite coulée et pour lequel une vitesse relative entre ladite lingotière et ladite coulée est nulle, ladite bande de temps positive définie comme la période de temps comprise dans lesdites périodes de déplacement ascendant et descendant dans lesquelles ladite vitesse verticale de la lingotière est relativement plus grande que ladite vitesse de retrait de ladite coulée et ladite bande de temps négative définie comme période de temps comprise dans lesdites périodes de déplacement ascendant et descendant dans lesquelles ladite vitesse verticale de la lingotière est relativement plus petite que ladite vitesse de retrait dudit métal coulé ;
rétraction desdites parois mobiles loin l'une de l'autre et pour cesser d'être en contact avec ledit moule mince lorsque ladite vitesse verticale de la lingotière peut s'appliquer à l'intérieur de ladite bande de temps positive, lesdites parois étant ouvertes à une première période de temps correspondant à l'endroit où ladite vitesse verticale de la lingotière se situe entre celle du point de début de ladite bande de temps positive et celle de ladite vitesse verticale maximum de la lingotière, à l'intérieur de ladite bande de temps positive,
lesdites parois mobiles étant fermées l'une vers l'autre et entrant en contact avec ledit moule mince à une deuxième période de temps correspondant à l'endroit où ladite vitesse verticale de la lingotière se situe entre celle de ladite vitesse verticale maximum, a l'intérieur de ladite bande de temps positive, et celle dudit point de fin de ladite bande de temps positive, ladite ouverture et ladite fermeture desdites parois auxdites première et deuxième périodes de temps se produisant à des vitesses égales à l'intérieur de ladite bande de temps positive ; puis
rétraction desdites parois mobiles loin l'une de l'autre et pour cesser d'être en contact avec ledit moule mince lorsque ladite vitesse verticale de la lingotière peut s'appliquer à l'intérieur de ladite bande de temps négative, lesdites parois étant ouvertes à une troisième période de temps correspondant à l'endroit où ladite vitesse verticale de la lingotière se situe entre celle du point de début de ladite bande de temps négative et celle de ladite vitesse verticale maximum de la lingotière, à l'intérieur de ladite bande de temps négative,
lesdites parois mobiles étant fermées l'une vers l'autre et entrant en contact avec ledit moule mince à une quatrième période de temps correspondant à l'endroit où ladite vitesse verticale de la lingotière se situe entre celle de ladite vitesse verticale maximum à l'intérieur de ladite bande de temps négative et celle du point de fin de ladite bande de temps négative, ladite ouverture et ladite fermeture desdites parois auxdites troisième et quatrième périodes de temps se produisant à des vitesses égales à l'intérieur de ladite bande de temps négative.
